

April 13, 1965

J. W. CLAPP ET AL

3,177,555

PROCESS FOR TREATING TEXTILE FILAMENTS

Filed Aug. 9, 1960

6 Sheets-Sheet 1



JOHN W. CLAPP  
ROBERT C. HART  
INVENTORS

BY *P. Frank Smith*  
*Harold N. Powell*  
ATTORNEYS

April 13, 1965

J. W. CLAPP ETAL

3,177,555

PROCESS FOR TREATING TEXTILE FILAMENTS

Filed Aug. 9, 1960

6 Sheets-Sheet 2



Fig. 2



Fig. 3

JOHN W. CLAPP  
ROBERT C. HART  
INVENTORS

BY *R. Frank Smith*  
*Howard N. Powell*

ATTORNEYS

April 13, 1965

J. W. CLAPP ET AL

3,177,555

PROCESS FOR TREATING TEXTILE FILAMENTS

Filed Aug. 9, 1960

6 Sheets-Sheet 3



**Fig. 5**



JOHN W. CLAPP  
ROBERT C. HART  
INVENTORS

BY *G. Frank Smith*  
*Harold N. Powell*

ATTORNEYS

April 13, 1965

J. W. CLAPP ETAL

3,177,555

PROCESS FOR TREATING TEXTILE FILAMENTS

Filed Aug. 9, 1960

6 Sheets-Sheet 4



JOHN W. CLAPP  
ROBERT C. HART  
INVENTORS

BY *R. Frank Smith*  
*Harold N. Powell*

ATTORNEYS

April 13, 1965

J. W. CLAPP ET AL

3,177,555

PROCESS FOR TREATING TEXTILE FILAMENTS

Filed Aug. 9, 1960

6 Sheets-Sheet 5

Fig. 7



JOHN W. CLAPP  
ROBERT C. HART  
INVENTORS

BY *R. Frank Smith*  
*Harold N. Powell*

ATTORNEYS

April 13, 1965

J. W. CLAPP ET AL

3,177,555

PROCESS FOR TREATING TEXTILE FILAMENTS

Filed Aug. 9, 1960

6 Sheets-Sheet 6



JOHN W. CLAPP  
ROBERT C. HART  
INVENTORS

BY *R. Frank Smith*  
*Harold N. Powell*

ATTORNEYS

1

3,177,555

**PROCESS FOR TREATING TEXTILE FILAMENTS**  
John W. Clapp and Robert C. Hart, Kingsport, Tenn.,  
assignors to Eastman Kodak Company, Rochester, N.Y.,  
a corporation of New Jersey

Filed Aug. 9, 1960, Ser. No. 48,443

3 Claims. (Cl. 28—72)

This invention relates to a process and apparatus for treating filaments. More particularly, this invention concerns a process and apparatus for treating tow made from filaments of a polymeric composition such as a tow composed of polyester type filaments.

It is well known that many types of filaments comprised of polymeric materials as produced by melt spinning or other methods do not possess the desired properties of strength, elongation, shrinkage or the like. Therefore, it is conventional practice in the industry to subject such polymeric filaments to various treatments including heating, stretching, setting and other steps for orienting the filaments and otherwise imparting improved properties thereto. Also, with respect to certain synthetic filaments which are suitable for use as produced, it is possible by stretching, setting and the like treatments in many instances to alter the properties of such filaments.

In order to accomplish the foregoing types of treatment such as stretching, setting and other comparable treatments, a large number of processes and apparatus have been proposed. Many of the prior art apparatus constructions have involved so-to-speak snubbing the filaments around small rolls or bars or pinching them between pinch rolls so that tension can be applied without the filaments unduly slipping. Such type of treatment where the filaments are pinched to any degree may be somewhat damaging to the quality of the yarn. Also in some of the apparatus, certain of the rolls have been heated in order to impart heat to the yarn being processed. However, it is apparent such type of heating may not be too uniform even though one surface of the yarn is first contacted with one heated roll and then another heated roll inasmuch as the surface of the yarn adjacent to the roll may become more heated than the outer surface of the yarn.

One rather simple, uncomplicated procedure which has been developed for treating filament yarn in the form of tow has comprised laying the filaments, usually in a crimped condition, upon a moving flat conveyor through which hot gas is passed. The tow is traversed onto the belt conveyor in order to obtain sufficient hold-up time in a heating unit of reasonable length. Shrinkage in such type process and apparatus is free and uncontrolled. There are also difficulties which may arise due to tangling and twisting of the filaments in the traversed tow. Also, in addition to the uncontrolled and nonuniform shrinkage, the filaments may lose crimp during the processing.

It is believed apparent, therefore, that the development of other methods and apparatus for the processing of yarn, tow and the like filamentary material represents a highly desirable result. After extended investigation, we have found a procedure and apparatus which it is thought is advantageous in several respects over prior art methods and apparatus, particularly in the capability of the process and apparatus of the present invention in producing a better filamentary material.

This invention has for one object a process for the after treatment of filamentary material to impart thereto improvement or desired properties. A particular object is to provide a process and apparatus that may be utilized for the treatment of and imparting enhanced properties to filamentary tow comprised of a polymeric material. A still further object is to provide a process

2

and apparatus of the class indicated which may be utilized for the treatment of filamentary tow comprised of a polyester composition. Another object is to provide a process of treating filamentary yarns and tows whereby may be produced a better and more uniform product.

5 Another object is to provide a process and apparatus of treatment of the class indicated where there will be fewer tangled, broken and displaced filaments. Still another object is to provide a process of treating filamentary products whereby the physical properties of the materials may be controlled at the desirable level by the improved control of shrinkage and fiber temperature. Another object is to provide a process and apparatus whereby the treated filamentary material may be suitable for use as continuous filament tow or cut staple. Still a further object is to produce a tow in which the resultant filaments are in a parallel arrangement without a substantial amount of tangled or broken filaments. Another and important object is to provide apparatus units and arrangements particularly adapted for carrying out the aforesaid process steps. Other objects will appear hereinafter.

A more complete understanding of our invention will be had by reference to the attached drawings forming a part of the present application.

25 FIG. 1 is a semidiagrammatic side elevation view in the nature of a flow sheet showing the arrangement of apparatus parts for carrying out our process. A number of the various units illustrated over-all in FIG. 1 will be described in greater detail in connection with certain of the other views;

30 FIG. 2 is a schematic perspective view of a flexible creel unit;

35 FIG. 3 is also a schematic side elevation view partly in section showing the over-all construction of a heating unit which may be used in our process.

40 FIG. 4 is a sectional view showing the interior construction of the heating unit of FIG. 3;

FIG. 5 is an end section of said heating unit;

45 FIG. 6 is a schematic perspective view of the over-all unit which may be employed in the present invention for treating our tow to impart uniform shrinkage characteristics and the like properties thereto. This figure is presented to show the unit with the side thereof removed;

50 FIG. 7 is likewise a schematic perspective view on a somewhat enlarged scale of one of the drums and associated parts of the series of the several drums shown in FIG. 6; and

55 FIG. 8 is a semidiagrammatic side elevation view of a device which may be used in our process for applying treating materials such as lubricant onto the filamentary tow being processed in our apparatus.

60 Referring to FIG. 1, 2 is a supply of the filamentary material which is to be treated. We prefer a somewhat flexible creel type of unit (as will be described in connection with FIG. 2) in order that various denier yarns and tows may be prepared and treated by our invention.

65 The filaments of the desired denier are withdrawn from unit 2 at 3 and passed below and around and over a plurality of rolls or drums 4, 5, 6, 7, 8 and 9. Preferably these drums are of about 1-2 feet in diameter and are positioned in the manner indicated in the drawing so that the filaments contact a substantial portion of the drum as, for example from about  $\frac{1}{2}$  to  $\frac{2}{3}$  of the surface of the drum. By employing such construction and arrangement,

70 the filaments are amply retarded so that substantial tension may be applied thereto without undue slippage. The filaments leaving the last of the feed rolls or drums at 10 pass into and through a heating unit 11. This heating unit will be described in greater detail in connection with FIGS. 3, 4 and 5; hence extended description at this point is unnecessary.

The heated filaments emerge at 12 then pass around

another series of rolls and drums 13, 14, 15, 16, 17 and 18. This further series of rolls is of the same or similar construction as the rolls already described, but are operated at a higher rate of speed. By this arrangement of a plurality of rolls about which the filamentary material is in substantial contact thereby resisting slippage, it is possible by speed differential of roll rotation to apply stretching, drafting, orienting and the like treatment to the filaments to any desired degree. In general we prefer to apply sufficient tension to the filaments so that they are elongated several hundred percent as for example two, two and one-half or three times their original length as measured at point 3.

The stretched or oriented filaments as at point 19 are then fed through the novel heat treating unit of the present invention indicated over-all at 21. Since this unit is described in detail in connection with FIGS. 6 and 7, extended description at this point is unnecessary. The further processed filaments at 22 are then passed through a device 24 where yarn treating materials may be applied prior to passing the filaments to a crimping operation at 25. The fully processed filaments emerging at 26 may then be passed to conventional cutters for manufacturing the materials into staple fiber from the continuous filament tow in which the filaments are relatively parallel. The tow may be passed to a tow packaging equipment (not shown) where the tow may be baled or otherwise packaged for certain uses.

The over-all arrangement of apparatus and its functioning is believed apparent to a substantial extent from the preceding description. However, a further understanding will be had from the following description which concerns the make-up of the several individual units comprising the over-all processing equipment.

Referring now to FIG. 2, we have a flexible creel for holding multiple units of the filamentary textile material which is to be processed by the present invention. Such units are comprised of the several individual stands 31, 32, 33, etc. which are adapted to be stacked one upon the other inasmuch as the legs of the stand are adapted to fit onto the legs of the other stands as indicated at 34. Each of these stands is adapted to contain several packages of yarn as indicated at 36, 37, and 38, for example. The exact number of yarn packages, the size of the filaments and the like do not constitute a limitation on the present invention. It is apparent from the existence of the large number of packages that it is possible to withdraw from as many of the packages as desired to make up a yarn or tow for processing as indicated at 39 of any desired denier. The yarn as withdrawn from the packages, passes through the several spring guides 40, 41 to and through the eye boards or bars 42 and 43 which means permit the yarn to move freely without undue tangling. Further eye boards may be provided at 44 so that additional filaments may be withdrawn in a similar manner and combined with the filaments at 39 to produce the yarn or tow of the desired denier.

In general in the operation of our process we would withdraw sufficient yarn from enough yarn packages to provide a tow of the order of 100,000 to 600,000 denier. Our apparatus as just described for supplying a source of tow to be treated by our process and apparatus is not only advantageous for providing flexibility for preparing a tow of the desired denier, but is useful in other respects. In the continuous operation of our process as one group of yarn packages becomes empty by the flexible arrangement of the present construction additional stands containing additional yarn may be stacked one upon the other adjacent to the eye boards and such yarn threaded through the retractable guides as 40 and 41 to provide a continuous supply of yarn.

The yarn strand or tow of several thousand denier as at 39 aforementioned, then passes under and around roll 4, 5, 6, etc. referred to above. As indicated by passing the band of filaments around and in substantial contact

with the several pairs of feed rolls 4-8 of FIG. 1, the yarn is positioned against slippage and may be drafted to the desired extent. In order to facilitate the drafting, it is desirable to heat the yarn as for example, to a temperature of the order of 100-225° C. This may be conveniently accomplished in a unit such as disclosed in FIG. 3.

Referring to FIG. 3, our heating unit is comprised of an elongated upper housing 51 and a similar lower housing 52. These sections are positioned slightly apart from each other in order to provide an elongated flat slot 53 through the unit so that the tow band may be passed therethrough. This elongated slot may be closed by the hinged door or cover 54.

Both the upper and lower sections are provided with heating coils 56 and 57, the construction of which will be more apparent from the description of figures which follow. Suitable inlet conduits are provided at 58 and 59 for supplying heating fluid such as steam to the apparatus. An exhaust duct is provided at 60 for the exhaust steam. A special inlet duct is provided at 61 for purposes of removing a mixture of steam and air from the end of the unit.

Referring now to FIG. 4, the various parts already referred to in connection with FIG. 3 are indicated thereon with the same numeral designations. As may be noted, the double baffle chambers 60, 61 and 61' on each end of the unit permit the inlet of fresh air which flows around the end of the unit in the chamber 61 and then through the yarn openings or slots 63 and 63' into the steam exhaust chambers 60 and 60'. This keeps the yarn slot 53 under slight suction and prevents the traveling yarn sheet from drawing in colder air and disturbing the heat balance within the unit.

In our preferred construction perforated plates are provided at 64 and 65 so that the super-heated steam entering at 66 and 67 is evenly distributed over reheating coils 68 and 69.

Referring now to FIG. 5, these reheating coils 68 and 69 may be better observed as well as the closure means 54. The strand or band of tow is suitably heated to, for example 100-225° C., in its passage through the elongated slot 53 and is stretched by the tension applied by the several draw rolls 13-18 referred to in FIG. 1. Since these draw rolls 13-18 and their positioning are substantially similar to feed rolls 4-8 already described, further description thereof appears to be unnecessary.

The band of tow which has now been suitably heated in the unit of FIGS. 3-5 just described and stretched by the higher speed or rotation of draw rolls 13-18 has now arrived at point 19 of FIG. 1 for processing in our new drum type heat setting equipment of FIGS. 6 and 7.

Referring now to FIG. 6, the drafted filaments at 71 are fed into our new heat setting apparatus over roll 72 and between guide rolls 73 and 74. The band of drafted filaments then passes around a plurality of drums 76, 78, 79, 80 and 81 in series. These drums are preferably of relatively large diameter so that the filaments are not subjected to bending at extreme angles. However, the width and diameter thereof may to some extent depend upon the size and number of filaments being processed. In general the drums would be of a diameter of 3-5 feet and of a width of from 1-2 feet.

Drums 77, 79 and 81 are positioned in a staggered offset relationship to drums 76, 78 and 80 so that the band of tow encircles or encompasses from 70% to 90% of the circumference of each drum. These drums have perforations around the entire surface periphery, such perforations being indicated at 83 and 84, for example. Internally of the drums there is provided a baffle as indicated at 86, 87 and 88 so as to close a portion of the perforations from the inside, namely the portion of the drum not covered by the band of tow on the outside. Depending upon the positioning of the drums and the like factors, baffles which cover  $\frac{1}{2}$  to  $\frac{1}{2}$  of the inner surface of the

drum are usually satisfactory. Generally a baffle which covers  $\frac{1}{4}$  of the interior surface is preferred.

The processed tow leaves the last drum 81 through guide rolls 91 and 92 thereby passing out of the apparatus to the spray lubricator 90. This series of drums is contained in an enclosed housing 93 so as to retain around the drums the heating medium that is supplied to the interior of the housing. This feature of supplying heating medium will be more apparent from FIG. 7. It will also be kept in mind that with respect to FIG. 6, the side of the housing has been removed in order to better show the arrangement of the drums within said housing.

Reference is made now to FIG. 7 which may be considered an illustrative two drum section out of the apparatus of FIG. 6. That is, the drums shown may be considered numbers 79 and 80 which have already been described above as positioned in housing 93. A wall member 94 is provided for fully enclosing the drums. There is also provided an internal wall member 96 for separating the chamber containing the several drums from the heating chamber 97. It will be noted that the drums are supported by a suitable enclosed support and mounting member 98 which serves not only to support the drums, but also as a closure or duct member so that the heating gas may be conducted out of the interior of the drums through openings 107 back into the heating chamber. The exact construction for mounting these several drums in a rotatable manner is not a limitation on the present invention and may be accomplished in any suitable manner. It is desired, however, that the driving means for the drums, whether by separate motors, belts, chain drives or the like, be such that the drums may be rotated at any desired speed of rotation, which speed of rotation may in some instances be the same for each drum or in other instances the drums may be operated at different speeds.

Heating chamber 97 which for clarity of disclosure has been shown open in FIG. 7, would be suitably closed for retaining the heat and gas circulation therein. Such chamber contains a heating unit 100 which may be in the form or any suitably radiated device. For example, unit 100 may comprise a steam radiator into which steam is introduced at 101 and condensate withdrawn at 102. Positioned above this heating unit is a partition or shelf member 103 which carries therein a suitable fan device 104. Positioned above this fan device are a plurality of baffles designated overall as 105 whereby the heated gaseous atmosphere may be deflected through opening 106 down onto the several drums 79 and 80. That is, a wall 96 referred to earlier has in the top a suitable opening for permitting the heating medium to circulate into the drum chamber. At the bottom of the wall there are provided suitable outlets 107. These outlets are connected by mounting member 98 with the interior of the drums so that circulation of the heating medium may be through the drum and back into the heating chamber.

With this type of heating medium circulation, the band of filaments on the drum are more thoroughly and uniformly heated while at the same time the gas circulation tends to produce pressure toward the surface of the drum thereby causing the filaments to better adhere to the drum surface. While the process and apparatus will be described with use of air as the heating medium, because of the enclosed nature of the construction, inert or other types of atmospheres may readily be utilized therein as for example, if an inert atmosphere is desired, the interior of the housing may be supplied with nitrogen.

Attention is now turned to FIG. 8 which discloses in some detail the spray lubricator device through which the filament band passes after leaving the heat setting apparatus. This processed filament band now designated 110 passes through device 111 wherein the filaments may have applied thereto various treatment agents exemplified by the following: 65% mineral oil, 25% diethylcyclohexylamine lauryl sulfate and 10% oleyl alcohol.

In further detail, still referring to FIG. 8, the treating

agents are contained in the reservoir 112 from which the treating materials flow through conduit 113 out of the spray atomizer 114.

This spray distributes the treating agent over the band of filaments, some of the treating agent being taken up by the filament band. The liquid not thus taken up by the filaments falls to the bottom of apparatus 111 and is collected in the dish or tapered collecting basins 116 and 117. The liquid thus collected passes through conduit 118 and is filtered at 119. The filtered liquid may then be circulated through conduits 121 and 122 to another spray atomizer 123 in the lower part of the unit. This spray atomizer positioned below the band of yarn permits the more complete treatment of the filaments with the treating agent.

The apparatus is provided with a suitable by-pass line 124 which leads to float chamber 125 thereby permitting the control of the liquid recycle. Suitable pumps may be provided at 126 and 127 for motivating the liquid through the device just described. After leaving the spray lubricator device, the band of filamentary material is then fed to crimper 130 (see FIG. 6) where filaments have imparted thereto a suitable uniform crimp. The crimped filaments may then be conducted to packaging and/or cutting devices for preparing staple fiber therefrom or other desired utilization of the filaments which have been processed in accordance with the present invention.

The operation of our process and the above described apparatus is thought to be apparent to a substantial extent from the foregoing description and drawings therein referred to. However, a still further understanding will be had from a consideration of the following examples.

#### Example I

In accordance with this example sufficient filaments were withdrawn from the packages thereof to provide a tow band of approximately 450,000 total denier after drafting and shrinking. This band which was of a width of about 18 inches was passed around the series of several feed rolls positioned in front of the heating unit. The band of tow was heated in the heating unit by steam to a temperature of 100-200° C. and the filaments drafted between 200% and 300%. The drafting was accomplished by passing the band of filaments around the series of draw rolls positioned beyond the heating unit. These draw rolls were operated at a sufficiently increased surface speed to produce the aforementioned drafting.

The drafted band of tow was then fed into the new heat-setting unit of the present invention, namely a unit in accordance with FIGS. 6 and 7. That is, the drafted band of tow was passed under and around a series of several perforated drums of a diameter of the order of 4½ feet which drums were contained in an enclosed chamber. The speed of rotation of the drums was synchronized with the speed of rotation of the drafting rolls so that the tow band was fed into the heat setting unit of the order of 10-25% greater speed than the surface speed of the drums. This permits normal shrinkage of the filaments to take place without substantial tension.

Although there is this 10-25% overfeed, the tow band is well held in place on the perforated drums by suction developed as high quantities of hot air (135°-220°) is circulated from the heating chamber through the drum perforations. This heated air moving from outside of the drums to the inside then back through the heating chamber where it is reheated, produces a small amount of reduced pressure which is adequate for maintaining the band of filaments on the drums in a relatively parallel untangled position.

As already described above, a portion of the interior of the drum periphery is sealed by the baffles 86, 87 and 88 referred to in FIG. 6 which prevent this reduced pressure acting upon the filaments between the discharge point and the pick-up point. By positioning the drums

relatively closely together and in an offset relationship as disclosed in FIG. 6, the drums will function in a self-threading manner.

After the tow band had passed around the several drums in series, it was discharged from the heat setting unit through the spray lubricator described in connection with FIG. 8 where the tow band was treated with a filament treating composition as described above.

From the tow treating chamber the band of tow passed continuously into a crimper where 8-12 crimps per inch were imparted to the tow. From the crimper the tow may be passed either to staple fiber manufacture or the continuous relatively untangled crimped tow may be delivered to packaging operations.

The method of the instant example exhibited certain advantages as follows. The crimp of the tow was better than with prior art processes where a crimping operation preceded the heat setting. It was necessary to crimp the tow to hold it together while it was passed through the flat bed dryer for heat setting. Since the heat setting operation removed a substantial amount of the crimp, a second crimper was required. By the present invention, the need of two crimpers is eliminated as well as associated parts. Also in the present process where the tow band is relatively straight and the filaments parallel, all the way through the process difficulties due to crossed and tangled filaments are eliminated thereby contributing to the production of a better crimped product.

By passing the tow band over rolls and drums of relatively large diameter, the filaments are not subjected to sharp bends which might impair the quality of the filaments. In addition, by the present invention it is possible to obtain a more uniform heating in a relatively short time thereby contributing to the enhanced quality of the crimped tow product.

#### Example II

In accordance with this example a tow of uncrimped polyester filaments of the order of 150,000 total denier was prepared in the form of a band of straight relatively parallel filaments. This band was heated and drafted substantially as described in connection with FIG. 1.

The drafted tow band was then fed into the drum unit at a speed of approximately 69 feet per minute which provides an overfeed of about 12%. The circulated gas temperature of the heating gas was at about 140° C. The circulation thereof through the drum perforations and over and around the tow band on the perforated drums very quickly and uniformly heated the filaments. The pressure drop of the heating gas across the perforated drums was approximately 2 inches of water. In this particular example the hold-up time in the drum apparatus was of the order of 14 seconds.

Tests of the resultant yarn produced by the present invention indicated properties of 2.9 grams per denier and a 25% elongation. Such properties were equal to the properties of comparable filaments treated by prior art procedure for 7 minutes at the same temperature.

#### Example III

In accordance with this example a 450,000 total denier uncrimped warp was processed. As in the preceding examples, the filaments were heated and drafted and then processed in the new heat setting unit of the present invention. In further detail, the drafted warp in the form of a band approximately 18 inches wide was passed through a six drum machine as illustrated in FIG. 6 at the rate of about 150 yards per minute with a 20% overfeed. This amount of overfeed compensated for the shrinkage of the polyester yarn. The gas temperature of the circulating gas within the heat setting unit was approximately 375° F. and this circulating gas very uniformly and quickly heated the filaments as well as provided with the reduced pressure for holding the band of filaments against the perforated drums. The tow re-

sulting had no objectionable tangled or crossed filaments as with conventional dryers, resulting in improved quality for processing on textile machinery.

#### Example IV

A modified polyacrylic tow of approximately 200,000 denier had been previously spun and drafted to attain properties as follows: 1.79 grams/denier tenacity, 25.7% elongation. Shrinkage in an oven at 125° C. was 12.4%.

When this tow was heat set in a conventional tow dryer at 150° C., it shrank 25-40%, with tight ends resulting from uneven shrinkage. Elongation increased to 47% with shrinkage in an oven at 125° C. negligible.

Use of the subject drum dryer on this tow enabled production of a tow at 9% shrinkage while heat setting at 155° C. The elongation only increased to 32% under these conditions, the shrinkage in an oven at 125° C. was still negligible and the condition of tight and loose ends was completely eliminated.

#### Example V

A yarn spun from polypropylene with an I.V. of approximately 1.0 was drafted at a ratio of 4.95 in superheated steam at 160° C. This yarn had properties as follows:

|                      |              |      |
|----------------------|--------------|------|
| Strength             | grams/denier | 3.90 |
| Elongation, percent  |              | 31.8 |
| Shrinkage at 125° C. |              | 8.6  |

The yarn was continually passed from the drafting operation through a six drum heat setting unit at 155° C. and a relax ratio of .875 and collected at 85 meters/minute. Properties were:

|                      |              |      |
|----------------------|--------------|------|
| Strength             | grams/denier | 3.08 |
| Elongation, percent  |              | 54.3 |
| Shrinkage at 125° C. |              | 4.0  |

The present invention has been described with particular reference to the treatment of polyester tows inasmuch as it is especially suitable for the processing of such material. Examples of polyester materials from which the filamentary tows may be prepared are disclosed in Bell, Kibler and Smith application Serial No. 544,639, now U.S. Patent No. 2,901,466. However, the process and apparatus of the present invention may be employed for the treatment of filamentary materials composed of other polymeric compositions. Illustrations of such other type filaments are as follows: polyacrylic, polypropylene, polyethylene and modified acrylic.

The amount of drafting applied to the filaments would be within the range of 200 to 1500%. The degree of heating the filaments during drafting would be within the range of 100° C. to 220° C.

Although we have described the heat setting operation with a certain percentage of overfeed, usually within the range of 10 to 30% and prefer such operation, however, it is possible to operate our process and apparatus so that the filaments may be further stretched rather than allowed to shrink if this is desired. That is, the surface speed of the perforated drums may be maintained equal with the speed of the drafting rolls or operated at a speed greater than the drafting rolls.

The gas used for heating is generally air, superheated steam or saturated steam as these are readily available heating mediums. However, any suitable heating medium may be used. In the event it is desired that the heat setting operation be conducted in the presence of inert atmosphere, the heating gas within the enclosed unit may be comprised of nitrogen, carbon dioxide, or a mixture of gases having low oxygen content.

Although the rolls and drums may be constructed of the usual materials of construction, we prefer that the surface of the feed rolls and drafting rolls be of stainless steel of a composition commercially obtainable as type 304 or 316. The perforated drums may be constructed

of stainless steel or other metals depending on the nature of the circulating gas, the fiber and the temperature used.

While we have described our invention as applicable to bands of filamentary material of several thousand total denier, our invention is applicable to material of total deniers within the range of 15,000 to 650,000. The denier per filament of the filaments treated may be within the range of 1.0 to 50. It is believed apparent from the foregoing description that it may be seen that this invention permits the production of improved yarns, tows, warps and the like for several reasons. The filamentary material is maintained in a relatively parallel condition. Crimping before heat treating is not necessary. In the present invention the heat treating occurs in less time and more uniformly as a result of the thin layer of filaments and the relatively high heating gas velocity that may be obtained. The filaments are maintained in place in parallel condition without the possibility of tangling by the suction in the perforated drum which is employed in our process.

The invention has been described in detail with particular reference to preferred embodiments thereof, but it will be understood that variations and modifications can be effected within the spirit and scope of the invention as described hereinabove and as defined in the appended claims.

We claim:

1. The process of treating a bundle of dry polymeric continuous filaments of a total denier within the range of 15,000 to 650,000, which comprises passing the bundle around a plurality of large diameter rolls in series so that the filaments contact at least about one-third of the diameter of the rolls, heating the filaments to 100-225° C. passing the heated filaments around a plurality of further rolls whereby the filaments contact at least one-third of the roll diameter of said further rolls, said further rolls being operated at a greater surface speed than the first group of rolls whereby the filaments are drawn, then shaping the drawn, dry filaments around a plurality of perforated drums of diameter of the order of 3-5 feet, said perforated drums rotating in a gaseous atmosphere heated to 135-220° C. whereby the gas circulates over

the dry, drawn polymeric filaments and into the interior of the drums through said perforations and thereby uniformly and relatively quickly heats the filaments and withdrawing the filaments from the last drum to further treatment.

2. The process of claim 1 wherein the further treatment includes applying a treating agent comprised of mineral oil, a sulfate and a long-chain unsaturated alcohol to the withdrawn filaments and then subjecting the filaments to a crimping operation.

3. The process of claim 1 wherein the dry polymeric continuous filaments treated consists essentially of a polyester composition.

15

#### References Cited by the Examiner

#### UNITED STATES PATENTS

|              |       |                   |         |
|--------------|-------|-------------------|---------|
| 2,142,718    | 1/39  | Dreyfus           | 28-59.5 |
| 2,321,635    | 6/43  | Taylor            | 28-59.5 |
| 20 2,444,064 | 6/48  | Philipp           | 28-59.5 |
| 2,520,202    | 8/50  | Frearson et al.   | 28-59.5 |
| 2,673,385    | 3/54  | Williamson et al. | 28-59.5 |
| 2,695,509    | 11/54 | Masich et al.     | 28-1    |
| 2,807,863    | 10/57 | Schenker          | 28-72   |
| 25 2,835,047 | 5/58  | Fleissner et al.  | 34-115  |
| 2,846,752    | 8/58  | Lessig            | 28-72   |
| 2,922,229    | 1/60  | Kiefer            | 34-115  |
| 3,028,653    | 4/62  | Evans             | 28-72   |
| 3,032,856    | 5/62  | Fleissner         | 28-59.5 |
| 30 3,043,018 | 7/62  | Fleissner         | 34-115  |

#### FOREIGN PATENTS

217,487 10/58 Australia.

35

#### OTHER REFERENCES

Linton: "The Modern Textile Dictionary," copyrighted 1954, published by Duell, Sloan, and Pearce—Little, Brown, and Company, New York.

40 MERVIN STEIN, *Primary Examiner.*

RUSSELL C. MADER, DONALD W. PARKER,  
*Examiners.*